

# UNITED STATES PATENT OFFICE.

FRITZ RETTIG, OF MULHOUSE, GERMANY.

## PROCESS OF MAKING COLORED DESIGNS ON WOVEN FABRICS.

SPECIFICATION forming part of Letters Patent No. 617,772, dated January 17, 1899.

Application filed September 27, 1897. Serial No. 653,246. (Specimens.)

*To all whom it may concern:*

Be it known that I, FRITZ RETTIG, of Mulhouse, Alsace, German Empire, have invented certain new and useful Improvements in the Production of Colored Designs on Woven Fabrics, of which the following is a specification.

This invention has reference to the production of colored designs on fabrics woven with embroidery-like patterns.

For some years fabrics have been woven so as to show raised designs, like embroidery-work, on a plain ground. The said fabrics are made in plain white and sometimes woven in colors, the white fabrics being dyed in plain colors, if desired, according to the usual methods. Imitations of fabrics woven in colors have been produced by printing so as to show white designs on a colored ground.

20 This has been effected by applying the color on the back of the material in the form of a thick paste, so that it may impregnate the ground, but not the raised or embroidered part, the fabric being then dried and fixed in the usual way—for example, by steaming.

Up to the present, however, it has not been found possible to produce woven fabrics having embroidery-like designs colored on the raised portion; and the object of the present 30 invention is the production of such colored fabrics.

In carrying out this invention a woven fabric is taken having thereon an embroidery-like design. This fabric should preferably 35 be entirely white; and the invention consists in applying to the raised design a different color to that of the ground.

According to one way of effecting the invention a resist is placed on the back of the 40 fabric, which is then dried, and then a new color is printed on the other side, which is fixed in the usual manner—for example, by steaming. As the resist prevents the color from being fixed in the ground, only the embroidery-like or raised parts of the fabric 45 eventually become colored. By washing, the resist and the unfixed color are removed, and a colored design is thus effectively obtained on a white or plain ground.

50 The invention can also be carried out by the discharge process. In this case the fabric is dyed with the color which it is eventu-

ally desired to obtain on the embroidery-like or raised portions. The back is then padded with the discharge and the fabric then passed 55 through the discharging-bath in the usual way, the result being that the dye is discharged, except that upon the raised portions.

Having stated the nature of the invention, 60 I will further illustrate it by giving the following examples; but I premise that these can be varied in their details and that they are merely typical, illustrating the application of the invention to particular cases: 65

Example 1: The back of the material is padded with thickened acetate of lime, dried, and the other side is then either padded or printed with an ordinary anilin-black, which is developed either by aging or short steaming. 70

Example 2: The back is padded with a tannin-color resist, (thickened antimony solution,) dried, and then there is printed on the other side a tannin color. The material is 75 then dried, steamed, and washed.

Example 3: The back is padded with a chrome or alum color resist, (citric or tar- 80 ic acid, sodium citrate,) dried, and then alizarin colors are padded or printed on the other side, followed by drying, steaming, and washing.

Example 4: The back is padded with a stan- 85 nous-salt resist, and then substantive azo colors are padded or printed on the other side, followed by drying, steaming, and washing.

Example 5: After padding the material with  $\beta$ -naphthol it is dried, padded, or printed on the back with a tin or sulfite resist, as de- 90 scribed before. The material is dried, and then there is padded or printed on the other side a diazo solution.

Example 6: The back is padded with a thickened sulfate-of-zinc solution, and there 95 are then printed on the other side pigment colors thickened by means of albumen.

I will now proceed to give examples of the manner in which the invention can be carried into practice, using the discharge method, as hereinbefore described. 100

Example 7: The material is dyed with indigo. The back is padded with thickened po- tassium chromate, dried, and passed through an oxalic-sulfuric-acid bath, washed, and

dried. By this means there are obtained blue raised designs on a white ground.

Example 8: The material is padded with tannin solution, which is fixed by means of 5 tartar emetic or antimony salt. Then the back is padded with thickened sodium hydrate. The material is then dried, steamed for from one to two minutes, passed through an acid-bath, (hydrochloric or sulfuric acid 10 of 2° to 4° Baumé,) washed, and dyed with tannin colors.

Example 9: The material is mordanted with chrome, iron, or aluminium mordants. The back is padded with a discharging paste, 15 (thickened tartaric or citric acid,) steamed for one to two minutes, or aged, passed through chalk and cow-dung baths, and dyed with alizarin colors.

Example 10: The material is dyed with 20 direct azo colors. The back is padded with thickened tin-salt discharge, followed by a steaming and washing.

It is possible by this invention to start with a fabric previously dyed in any single color, 25 the effect being that the new colored designs are on a colored ground; but care must be taken that the coloring-matter on the dyed fabric originally taken does not interfere with the action of the resist.

30 A more practical method of producing colored raised designs on colored grounds is to incorporate in the resist a suitable coloring-matter. For example, the back of the fabric may be padded or printed with a tannin-color 35 resist, which contains substantive azo colors, and then dried. The right side of the fabric is then printed or padded with tannin colors, dried, steamed, and washed. In this way colored raised designs are obtained on a colored ground. The same effect can also be obtained by following example 1 and incorporating a coloring-matter with the thickened 40 acetate of lime. In this case a black raised design is obtained on a colored ground.

In carrying out this invention the back of 45 the material may be padded with a resist of such composition and strength as to be only able to reserve a part of the colors, which are padded or printed on the other side, thus making more than one color or shade in ad- 50 dition to the ground.

What I claim, and desire to secure by Letters Patent, is—

1. The improved process of producing embroidery-like woven material having a raised 55 and colored portion, which process consists in weaving such fabric with a raised design on its face, applying color to the face of the fabric, protecting the back and ground of the fabric from the applied color, fixing the color 60 on the face of the raised portion, and removing the unfixed color.

2. The process of coloring embroidery-like woven material woven with a raised pattern on its face, which process consists in protecting the back of the fabric by applying a resist thereto, applying a color on the other side, fixing said color on the raised pattern, and subsequently removing the resist and unfixed color.

3. The process of coloring embroidery-like woven material woven with a raised pattern on its face, which process consists in applying to the back of the fabric a resist having incorporated therewith a suitable coloring- 75 matter, in then applying an appropriate coloring-matter to the front of the fabric, fixing the color of the ground and that of the raised pattern and removing the resist and unfixed color.

In witness whereof I have hereunto signed my name in the presence of two subscribing witnesses.

FRITZ RETTIG.

Witnesses:

ROBERT WAGNER,  
MAX KOEHNLEIN.